

## UNITED STATES PATENT OFFICE

2,342,277

SEPARATION OF PYRITE, ARSENOPYRITE,  
AND PYRRHOTITE BY FLOTATIONEarl C. Herkenhoff, Stamford, Conn., assignor to  
American Cyanamid Company, New York,  
N. Y., a corporation of MaineNo Drawing. Application February 2, 1943,  
Serial No. 474,491

4 Claims. (Cl. 209—167)

This invention relates to a process of separating pyrite from arsenopyrite and/or from pyrrhotite by froth flotation.

Many sulfide ores contain mixtures of pyrite and arsenopyrite and in some cases mixtures of pyrite, arsenopyrite and pyrrhotite. It is desirable to obtain concentrates of the minerals separately because of the different uses to which the minerals may be put. Thus, for example, if pyrite is to be burned to sulfadioxide for the production of sulfuric acid by the contact process the presence of arsenic is undesirable and pyrite containing considerable amounts of arsenopyrite is not suitable for this purpose. The mixed ores may in some cases contain precious metal values, particularly gold or silver, and it is common in such cases for the precious metals to be primarily associated with the arsenopyrite. Inasmuch as the precious metal content of such ores frequently represents a considerable portion of the values it is important to obtain a concentrate which contains a large portion of the arsenopyrite.

It has been proposed in the past to depress one or other of the minerals by the addition of agents such as lime or sodium cyanide. These procedures do result in some separation but the separation is not sharp and leaves much to be desired.

According to the present invention froth flotation is effected after conditioning with a small amount of a permanganate such as sodium or potassium permanganate. The permanganate depresses the arsenopyrite and pyrrhotite, whereas pyrite is but little affected and can thereafter be recovered as a concentrate by froth flotation. In the case of ores containing only pyrite and arsenopyrite this procedure results in a satisfactory practical process.

It has further been found that the depressing action of the permanganate is not the same for arsenopyrite and pyrrhotite, the pyrrhotite being more readily depressed than the arsenopyrite. It is, therefore, possible to effect a separation of the three minerals by first conditioning with a smaller amount of permanganate which is sufficient to substantially depress pyrrhotite without depressing any considerable portions of arsenopyrite. Froth flotation will then result in

producing a concentrate containing pyrite and arsenopyrite which can then be conditioned with larger amounts of permanganate and again floated to produce a pyrite concentrate.

5 The amount of permanganate used will, of course, vary with the nature of the ore and with the relative contents of arsenopyrite and pyrrhotite. In general a satisfactory depression of arsenopyrite is obtainable with amounts of permanganate of the order of a quarter of a pound per ton or less. Selective depression of pyrrhotite without depressing arsenopyrite will ordinarily require amounts of permanganate less than 0.05 pound per ton.

10 It is an advantage of the present invention that the flotation operation on the conditioned pulp is not critical and the normal sulfide flotation reagents may be used such as xanthates, dithiophosphates, mercapto-benzothiazoles, and the like. While ordinary sulfide reagents may be used, they differ somewhat in effectiveness, and I have found that the best results are obtained with dithiophosphoric acids, dithiophosphates, or mixtures of dithiophosphates with mercapto-benzothiazole and reagents of this type are preferred.

15 The invention will be described in greater detail in conjunction with the following specific examples. The parts are by weight.

## EXAMPLE 1

An ore containing pyrite, arsenopyrite and pyrrhotite, associated with a gangue which also contained iron and sulfur, was treated for high arsenopyrite recovery. The arsenic content represented the major value of the ore under present economic conditions. The ore was first subjected to a bulk sulfide flotation with stage oiling using dicesyldithiophosphoric acid and sodium isopropyl xanthate as promoters. The concentrate was then conditioned with 0.02 lb. of potassium permanganate and floated in two stages using a small additional amount of the dicesyldithiophosphoric acid. The purpose of the flotation was to produce a pyrite-arsenopyrite concentrate with a maximum rejection of the pyrrhotite. The sequence of conditioning and amounts of re-

agents, together with metallurgical results, appear in the following two tables:

benzothiazole - disecondarybutyldithiophosphoric acid reagent.

*Conditions and reagents*

| Point of addition | Conditions    |                 |      | Reagents, pounds per ton |                                 |       |      |                   |
|-------------------|---------------|-----------------|------|--------------------------|---------------------------------|-------|------|-------------------|
|                   | Time, minutes | Per cent solids | pH   | CuSO <sub>4</sub>        | Na <sub>2</sub> CO <sub>3</sub> | AF 15 | 343  | KMnO <sub>4</sub> |
| Condition         | 3             | 23              |      | 0.50                     | 4.0                             |       |      |                   |
| Do                | 1/2           | 23              | 10.6 |                          |                                 | 0.117 | 0.05 |                   |
| Flotation         | 1/2           |                 |      |                          |                                 | 0.078 | 0.05 |                   |
| Condition         | 1/2           |                 |      |                          |                                 |       |      |                   |
| Flotation         | 1/2           |                 |      |                          |                                 |       |      |                   |
| Cond. concentrate | 1/4           | 1.5             |      |                          |                                 |       |      | 0.020             |
| Cl. flotation     | 1             |                 |      |                          |                                 |       |      |                   |
| Do                | 1             |                 |      |                          |                                 | 0.039 |      |                   |

The promoters are referred to by trade designation. "AF 15" is dicesyldithiophosphoric acid diluted with cresols. "343" is sodium isopropyl xanthate.

*Metallurgical results*

*Metallurgical results*

| Product            | Weight   | Assays   |          |          |
|--------------------|----------|----------|----------|----------|
|                    |          | As       | Fe       | S        |
|                    | Per cent | Per cent | Per cent | Per cent |
| Head               | 100.00   | 0.24     | 15.95    | 3.28     |
| Clean, concentrate | 1.64     | 12.50    | 42.90    | 37.62    |
| Clean, Tail        | 4.29     | 0.64     | 43.58    | 26.50    |
| Rgh. Tail          | 94.07    | 0.006    | 14.22    | 1.62     |

It will be apparent that a very effective depression of pyrrhotite took place and a major portion of the arsenic was recovered in a relatively high grade arsenopyrite-pyrite concentrate. When the same procedure was carried out but the potassium permanganate conditioning omitted the cleaner concentrate contained only 4.56% of arsenic and but little rejection of pyrrhotite took place.

*EXAMPLE 2*

An ore similar in nature to that of Example 1 was subjected to the same type of treatment as described in Example 1, but the cleaner concentrate was then further conditioned with additional potassium permanganate and subjected to a third flotation. The additional permanganate which acted as a depressant required further addition of collectors and frothers, the additional collector being a mixture of the sodium salts of mercaptobenzothiazole and disecondarybutyldithiophosphoric acid. The flotation procedure and arsenic assays appear in the following tables:

| Product     | Assays |           |          |          | Per cent weight As |
|-------------|--------|-----------|----------|----------|--------------------|
|             | Head   | Py. Conc. | As Conc. | Cl. Tail |                    |
| 25          | 100.00 | 0.51      | 0.33     | 1.13     | 18.10              |
| Py. Conc.   |        |           |          | 3.59     | 0.37               |
| As Conc.    |        |           |          | 94.71    | 0.015              |
| Cl. Tail    |        |           |          | 1.70     | 12.77              |
| Rgh. Tail   |        |           |          | 5.29     | 4.36               |
| Comb. Conc. |        |           |          |          |                    |
| Rgh. Conc.  |        |           |          |          |                    |

30 It will be apparent that a high degree of concentration of arsenopyrite was obtained, 84 to 1, and the pyrite concentration was even higher, amounting to 196 to 1.

35 A blank test which followed the same sequence but omitted the potassium permanganate conditioning gave an arsenopyrite concentrate having only 1.17% of arsenic, more than 92% of the arsenopyrite remaining in the pyrite concentrate.

30 Flotation operations in the examples were carried out under standard conditions using Fagergren flotation machines and operating conditions such as air and the like were the same for both blank tests and those using permanganate conditioning.

40 45 In the examples potassium permanganate has been described because of its ready availability. sodium permanganate gives the same result and in large scale use presents some economies.

I claim:

50 1. A method of separating pyrite from arsenopyrite which comprises subjecting a mixture containing both to conditioning with a sufficient alkali metal permanganate to depress the arsenopyrite and subjecting the conditioned material to 55 froth flotation in the presence of a promoter for

*Conditions and reagents*

| Point of additions | Conditions    |                 |     | Reagents, pounds per ton |                                 |       |      |                   |       |      |
|--------------------|---------------|-----------------|-----|--------------------------|---------------------------------|-------|------|-------------------|-------|------|
|                    | Time, minutes | Per cent solids | pH  | CuSO <sub>4</sub>        | Na <sub>2</sub> CO <sub>3</sub> | AF 15 | 343  | KMnO <sub>4</sub> | P. O. | 404  |
| Condition          | 3             | 23              |     | 0.50                     | 4.0                             |       |      |                   |       |      |
| Condition          | 1             | 23              | 9.4 |                          |                                 | 0.117 | 0.05 |                   |       |      |
| Rgh. flotation     | 2             | 23              |     |                          |                                 |       |      |                   |       |      |
| Cond. Rgh. Conc.   | 1/2           | 1.5             |     |                          |                                 |       |      |                   | 0.015 |      |
| Clean. flotation   | 2             |                 | 7.4 |                          |                                 | 0.039 |      |                   |       |      |
| Cond. Cl. Conc.    | 10            | 1.0             |     |                          |                                 |       |      |                   | 1.00  |      |
| Cond. Cl. Conc.    | 1             |                 |     |                          |                                 |       |      |                   | 0.054 | 0.03 |
| Py. flotation      | 3             |                 | 5.5 |                          |                                 |       |      |                   |       |      |

19.02 added at 5 minutes.

The promoters are referred to by trade designation. "AF 15" is a dicesyldithiophosphoric acid diluted with cresols. "343" is sodium isopropyl xanthate. "P. O." stands for pine oil and "404" for an undiluted mixed sodium mercapto-

pyrite, whereby a concentrate is obtained rich in pyrite and a tailing rich in arsenopyrite.

2. A method of separating pyrite, arsenopyrite and pyrrhotite which comprises subjecting a mixture containing the three minerals to condition-

ing with a small amount of an alkali metal permanganate sufficient to depress the pyrrhotite but insufficient to substantially depress the arsenopyrite, subjecting the conditioned material to froth flotation in the presence of a sulfide promoter whereby a concentrate is produced rich in pyrite and arsenopyrite and the tailing containing most of the pyrrhotite, conditioning the concentrate with an additional amount of alkali metal permanganate sufficient to depress the arsenopyrite and subjecting the conditioned material to froth flotation in the presence of a sulfide col-

lector whereby a concentrate is produced rich in pyrite and a tailing containing the arsenopyrite.

3. A method according to claim 1 in which the froth flotation takes place in the presence of a collector containing the dithiophosphoric acid radical.

4. A method according to claim 2 in which both flotation operations are effected in the presence of a collector containing the dithiophosphoric acid radical.

EARL C. HERKENHOFF.